

1

2,698,795

**SULFAMYL COUPLERS IN MIXED PACKET PHOTOGRAPHIC EMULSIONS**

Homer W. J. Cressman and Scheuring S. Fierke, Rochester, N. Y., assignors to Eastman Kodak Company, Rochester, N. Y., a corporation of New Jersey

No Drawing, Application March 26, 1953,  
Serial No. 344,894

6 Claims. (Cl. 95—2)

This invention relates to color photography and particularly to mixed packet photographic emulsions.

There have been many prior suggestions of mixed grain photographic emulsions, that is, photographic systems in which differently sensitized silver halide grains are incorporated in a single photographic emulsion layer and used to produce differently colored photographic images in the layer. Mixed grain systems have a number of advantages, chief among which is the simplicity of coating a single emulsion layer rather than several layers. Other advantages are the improved definition obtained by having the differently sensitized particles juxtaposed in a single layer, and the simplification of processing which is generally obtained.

It is sometimes advantageous to incorporate color forming compounds or couplers of the water-soluble type either in multilayer or mixed packet emulsions. Such couplers should be non-diffusing, particularly in mixed packet emulsions, but should possess sufficient reactivity in the color forming reaction to yield adequate dye densities.

It is therefore an object of the present invention to provide a novel incorporated coupler emulsion. A further object is to provide a method of incorporating couplers in silver halide emulsions. A still further object is to provide a novel mixed packet emulsion. Other

15

25

20

25

30

35

40

objects will appear from the following description of our invention.

These objects are accomplished by incorporating a particular type of coupler in a colloid-silver halide emulsion in the presence of a water-soluble salt of a polymer containing salt forming acid groups, e. g. a methylmethacrylate-methacrylic acid copolymer, bringing the pH of the mixture to a point below 7 immediately after adding the polymer, and adding a packet-forming component, e. g. a styrene-maleamic acid copolymer, to form particles of colloid packet-forming component and silver halide, containing the coupler.

The couplers which we propose to use are couplers or color forming compounds capable of reacting with the oxidation product of a primary aromatic amino developing agent on photographic development, containing one or more of the following groups: sulfamylbenzamido, di-sulfamylbenzamido, alkylsulfamylbenzamido, di-alkylsulfamylbenzamido, aminoalkylsulfamylbenzamido, di-aminoalkylsulfamylbenzamido, hydroxyalkylsulfamylbenzamido, or dihydroxyalkylsulfamylbenzamido.

These couplers have the general structure:



where

Z=a coupler

R<sub>1</sub>, R<sub>2</sub>=hydrogen, alkyl, aminoalkyl or hydroxyalkyl,  
e. g. hydroxyethyl

X=hydrogen or



The following couplers are suitable for use according to our invention:

(1)



1 - hydroxy - 4 - chloro - N - {4' - [2'' - (2'''', 4''' - di - tert - amylphenoxy) - 5'' - (3'''', 5''' - di - β - hydroxyethylsulfamylbenzamido)benzamido]phenethyl}-2-naphthamide.

(2)



1 - hydroxy - 4 - chloro - N - {4' - [2'' - (2'''', 4''' - di - tert - amylphenoxy) - 5'' - (3'''', 5''' - [di(di - β - hydroxyethylsulfamyl)]benzamido]phenethyl}-2-naphthamide.



(3)



1 - hydroxy - 4 - chloro - N - {4' - [2' - (2'',4'' - di - tert - amyloxy) - 5' - (3'',5'' - bis{N - [try(hydroxymethyl)methylsulfamyl)benzamido]phenethyl} - 2 - naphthamide.

(4)



1 - hydroxy - 4 - chloro - N - {4' - [2' - (2'',4'' - di - tert - amyloxy) - 5' - (3'',5'' - bis{N - [1,1 - di(hydroxymethyl)ethylsulfamyl)benzamido]phenethyl} - 2 - naphthamide.

(5)



45

1 - hydroxy - N - {β - {3 - [bis(β-hydroxyethyl)sulfamyl]benzylamido}ethyl}-4-chloro-2-naphthamide.

(6)



1 - hydroxy - N - {p - {2 - (2,4 - di - tert - amyloxy) - 5 - {m - [tris (hydroxymethyl) methyl] sulfamylbenzamido}benzamido}phenethyl)-2-naphthamide.

(7)



1 - hydroxy - 4 - chloro - N - {p - {2 - [2,4 - di - tert - amyloxy] - 5 - [m - (β - hydroxyethylsulfamyl)benzamido]phenethyl} - 2 - naphthamide.

5



1 - hydroxy - N - {p - {5 - {m - [bis(β - hydroxyethyl)sulfamyl]}-benzamido - 2 - 2,4 - di - tert - amylphenoxy}benzamido}phenethyl} - 4 - chloro - 2 - naphthamide.

(9)

1 - hydroxy - 4 - chloro - N - { $\beta$  - {2 - [2,4 - di - tert - amylophenoxy] - 5 - [m - ( $\beta$  - hydroxyethylsulfamyl)benzamido]benzamido}ethyl}-2-naphthamide.

1 - hydroxy - N - { $\beta$  - {5 - {m - [bis( $\beta$  - hydroxyethyl)sulfamyl]benzamido} - 2 - {2,4 - di - tert - amylophenoxy}benzamido}ethyl} - 4 - chloro - 2 - naphthamide

2,4 - dichloro - 6 - {2' - {2'',4'' - di - tert - amylophenoxy} - 5' - [3'' - (β - hydroxyethylsulfamyl)benzamido]benzamido} - 3 - methoxyphenol.

1 - phenyl - 3 - {3' - [2' - (2''' , 4''' - di - tert - amylophenoxy) - 5' - (3''' , 5''' - di -  $\beta$  - hydroxyethylsulfamylbenzamido)benzamido]benzamido} - 5 - pyrazolone.

7



8



17)



18)



19)



20)



(21)



$\alpha$  - (o - methoxybenzoyl) - 4 - {5 - {3 - [bis( $\beta$  - hydroxyethyl) - sulfamyl]benzamido} - 2 - {2,4 - di - tert - amylophenoxy} - benzamido}acetanilide.

SO<sub>2</sub>N(CH<sub>2</sub>CH<sub>2</sub>OH)<sub>2</sub>

(22)



$\alpha$  - (o - methoxybenzoyl) - 4 - {2' - [2,4 - di - tert - amylophenoxyl] - 5' - [ $\beta$  - hydroxyethylsulfamyl]benzamido}benza-  
mido)acetanilide.

The silver halide emulsions in which these couplers are incorporated may be optically sensitized and ordinarily two or more emulsions sensitive to different regions of the visible spectrum will be employed and mixed.

The coupler may be made in dispersion in gelatin or in solution in water, added to the silver halide emulsion or to the water-soluble salt such as the salt of methylmethacrylate-methacrylic acid copolymer, and then the remaining component that is, either the water-soluble salt or the silver halide emulsion, added to the mixture.

The water-soluble salt of the polymeric material containing salt-forming acid groups which is employed in forming the emulsion may be a salt obtained from the copolymer of methacrylic acid and methyl- $\alpha$ -methacrylate (Minsk, Weyerts and McDowell U. S. Patent 2,391,181), algin (alkali metal salt of polymeric-d-mannuronic acid), carboxymethyl cellulose (Collins, Freeman and Anthonisen U. S. Patent 2,278,612), or cellulose sulfate (Belgian Patent 448,249). The water-soluble polymer when mixed with the gelatin of the dispersion acts as a modifying agent so that small packets containing appropriately sensitized silver halide and color-forming coupler can be formed.

The polymeric packet-forming component consists of a polymeric carbon chain having recurring phenyl groups and carboxylic acid groups and preferably also carboxylic acid amide groups or imide groups or both and is used as the water-soluble salt such as the ammonium, sodium, potassium or lithium salt. The polymeric packet-forming component is preferably an interpolymer of styrene and an  $\alpha, \beta$ -unsaturated carboxylic acid, part of whose carboxyl groups may have been converted to amide or imide derivatives or both, such as interpolymers of styrene-maleic acid, styrene-acrylic acid, styrene-methacrylic acid, or styrene-itaconic acid.

The packet emulsion in its single layer or single color form consists of particles or packets of gelatin associated with polymeric packet-forming component containing silver halide and coupler, the packets being dispersed in an aqueous medium containing additional gelatin or another film-forming water-soluble polymer. To make a mixed packet emulsion this single emulsion is mixed with at least one other similarly made packet dispersion containing differently sensitized silver halide and different coupler to form the finished mixed packet emulsion.

In the preparation of the system described above, that is, gelatin, water-soluble polymer, and packet-forming component, the ingredients must be present in a

fairly definite ratio. If the gelatin is present in approximately 0.7% aqueous solution (an appropriate concentration for making an emulsion), then the water-soluble polymer should be present in an amount from about 1 to 2 times that of the gelatin, and the packet forming component should be present in an amount from 0.01 to 0.5 times that of the gelatin. Within these ranges the three-component systems exhibit a definite degree of optical turbidity. If this turbidity is measured in optical density per cm. of mixture at 30° C., using orange-colored light, of about 5800 A. U., the optical density is greater than 0.05, and is generally of the order of 0.1.

Suitable polymers of styrene with maleic acid or its derivatives which may be used as the polymeric packet-forming component according to our invention are described in Godowsky U. S. application Serial No. 156,066, filed April 15, 1950. The polymers illustrated in Examples 2 and 3 of the Godowsky application are especially suitable for use according to our invention.

The hydroxylalkyl sulfamyl couplers which we use were prepared in general by treating the parent coupler containing a chlorinated sulfonic acid group or groups with the appropriate amine. The preparation is described in detail in Salminen and Weissberger U. S. application Serial No. 344,884, filed concurrently here-with.

The following two examples describe preparation of the coupler dispersions in gelatin.

*Example 1.—Dispersion in gelatin of Compound 1*

An intimate mixture of 9.92 g. of 1-hydroxy-4-chloro-N - {4' - [2" - (2'''4''' - di - tert - amylo) - phenoxy - 5" - (3'''5''' - dichlorosulfonyl)benzamido] - benzamido} - phenamyl-2-naphthamide, 20.0 cc. of methanol, and 4.0 cc. of monoethanolamine, after the first vigorous exothermic reaction had subsided, was heated to 55° C. The clear solution, after 15 minutes at 55° C., was poured slowly into a mechanically agitated solution of 75.0 g. of a 10% deashed gelatin solution, and 5 cc. of a 5% Alkanol B solution. The mixture was milled 5 times through a colloid mill, chilled, shredded, and washed in 5 changes of 800 cc. of water; the first and second portions contained respectively 8 cc. and 5 cc. of a 20% acetic acid solution to take out excess ethanolamine. The washed noodles and 5 cc. of a 5% Alkanol B solution were stirred for 30 minutes at 40° C. and finally passed five times through the colloid mill set at .010". The weight of the coupler dispersion 85 was 185 g.

*Example 2.—Dispersion in gelatin of Compound 14*

A mixture of 4.73 g. of 1-phenyl-3-{3'-(2'',4''-di - tert - amylphenoxy) - 5''(3'',5'' - dichlorosulfonyl) - benzamido} - benzamido - 5 - pyrazolone, 20 cc. of methanol, and 5 cc. of monoethanolamine was heated to 55° C. and maintained at that temperature for 10 minutes. The dark brown solution was then slowly poured into 1000 cc. of cold tap water, vigorously agitated. The colloidal precipitate, after acidification (pH 6.5) of the aqueous mixture, was collected on a Buchner funnel, washed a second time by stirring in 500 cc. of distilled water, was sucked as dry as possible on the filter. It was then stirred into 25.0 g. of a deashed 10% gelatin solution, 25 cc. distilled water, and 5 cc. of a 5% Alkanol B solution. The coupler-gelatin mixture was passed five times through the colloid mill set at .010". The weight of the dispersion was 95.0 g.

Packet emulsions were prepared from the coupler dispersions in gelatin as follows:

*Example 3*

A mixture of 21.3 g. of the coupler dispersion described in Example 1, 39.6 g. of a red-sensitive emulsion, (containing permole of silver halide 80.0 g. of gelatin in a total weight of 1320 g.), and 25.0 cc. of distilled water was stirred at 40° C. for 5 minutes. The above components had been preheated to 40° C. prior to mixing. To this well-stirred, intimate mixture was then added 70.0 g. of a 10% solution of a copolymer of methyl methacrylate and methacrylic acid. The pH of this mixture, after stirring for 5 minutes at 40° C., was adjusted to 6.6 by slowly adding 5 cc. of a 10% citric acid solution. After the addition of 5.0 cc. of a 5% Alkanol B solution, the above mixture was moderately stirred at 40° C. for 20 minutes. To this intimate mixture was then added all at once 29.0 cc. of a 1% solution of styrene-maleamic acid copolymer, preheated to 40° C. The whole was vigorously stirred for 5 minutes and moderately stirred for another 18-20 minutes, then the packet reaction was complete. The well-defined particles averaged approximately 5μ in size. There was no free silver halide in the matrix on testing by microscopic examination a portion of the reaction mixture in a 5% gelatin solution.

The cyan packet emulsion prepared in this manner, after the addition of 75 cc. of 10% deashed gelatin solution and 5 cc. of a 7.5% saponin solution, weighed 275.0 g.

*Example 4*

A magenta packet emulsion was prepared similarly to Example 3, from 21.2 g. of the coupler dispersion described under Example 2, 27.6 g. of a green-sensitive emulsion (1370 g. per mole of silver halide and 80 g. of gelatin), 30 cc. of water, 48 cc. of a 10% solution of a copolymer of methyl methacrylate and methacrylic acid, 4.0 cc. of a 10% acetic acid solution, 3.2 cc. of a 5% Alkanol B solution, 20.0 cc. of a 1% solution of styrene-maleamic acid copolymer, 50.0 cc. of a 10% deashed gelatin solution, and 5.0 cc. of a 7.5% saponin solution. The magenta packet emulsion weighed 198.0 g.

Packet emulsions were prepared from the crystalline couplers (i. e., not dispersed in gelatin) as follows:

*Example 5*

A mixture of 20.0 g. of Compound 1, 30.0 cc. of methanol, and 2.0 cc. of a 20% aqueous sodium hydroxide solution was stirred at 60° C. for 5 minutes. To this almost clear solution was then added 48.0 cc. of water, and the whole stirred at 55-60° C. for another 15 minutes. The coupler solution (100 cc.) was filtered and 90.0 cc. of the filtrate, containing 18.0 g. of the cyan coupler No. 1, was added with efficient mechanical stirring to 204.0 g. of a 9.8% solution of a copolymer of methyl methacrylate and methacrylic acid (40° C.). To this mixture, after stirring for a minute or two at 40° C., was added slowly 22.8 cc. of a 10% citric acid solution and then stirred for 10 minutes. To this mixture was added 79.2 g. of a red-sensitive emulsion, (containing per mole of silver halide 80 g. of gelatin in a total weight of 1320 g.), 40.0 cc. of water and 6.0 cc. of a 5% Alkanol B solution. Into this mixture, after stirring at 40° C. for 30 minutes, was poured from a graduate 48.0 cc. of a 1% solution of a styrene-maleamic acid copolymer, preheated to 40° C. The whole was vigorously stirred

for the first 5 minutes and then moderately for another 25 minutes. A 10% solution of a deashed gelatin (180.0 cc.) and 20 cc. of a 7.5% saponin solution were then added.

5 The cyan packet emulsion prepared in this manner weighed 685 g. The average particle size was 5 to 8μ with a few clumps as high as 15μ.

*Example 6*

10 A magenta coupler solution was prepared from 18.0 g. of Compound 14, 30.0 cc. of methanol, 3.0 cc. of a 20% sodium hydroxide solution, and 149.0 cc. of water.

The magenta packet emulsion was prepared according to the procedure described in detail under Example 5.

15 The various components used were:

|                                                                                    |    |       |
|------------------------------------------------------------------------------------|----|-------|
| Magenta coupler solution                                                           | cc | 200   |
| 10% solution of a copolymer of methyl methacrylate-methacrylic acid                | g  | 168.0 |
| 10% citric acid solution                                                           | cc | 27.0  |
| 20 Green-sensitive emulsion (weight per mole silver halide 1380 g., gelatin 80 g.) | g  | 97.0  |
| Water                                                                              | cc | 40.0  |
| 5% Alkanol B                                                                       | cc | 7.0   |
| 25 10% solution of styrene-maleamic acid copolymer                                 | cc | 70.0  |
| 10% solution deashed gelatin                                                       | cc | 210.0 |
| 7.5% saponin solution                                                              | cc | 33.0  |

The total weight of the magenta packet emulsion prepared in this manner amounted to 800.0 g.

A two-color mixed packet emulsion was made as follows:

Example 7.—The mixed emulsion was made by mixing the following ingredients in the order stated:

|    |        |                                                                                    |
|----|--------|------------------------------------------------------------------------------------|
| 35 | 33.0   | g. of cyan emulsion (Ex. 3)                                                        |
|    | 14.0   | g. of magenta emulsion (Ex. 4)                                                     |
|    | 0.378  | g. of diethyl hydroquinone dissolved in dibutyl phthalate and dispersed in gelatin |
| 40 | 0.0043 | g. of benzothiazole methiodide in 2.6 ml. of methanol                              |
|    | 0.8    | cc. of a 20% KCl, 2% KBr solution                                                  |
|    | 1.0    | cc. of a 7.5% saponin solution                                                     |
|    | .008   | g. of mucochloric acid in 0.3 cc. of water                                         |

45 60.0 g. total

The red and green exposed areas of these plates on processing in a primary aromatic amino color developing solution yielded respectively cyan and magenta dye images of satisfactory color density. The color separation was quite good.

Numerous modifications may be made in the packet systems within the scope of our invention. In a multi-layer film one or more couplers may be incorporated in 55 packets and the remaining coupler or couplers may be incorporated in separate layers in dispersion in a coupler solvent or directly incorporated in the gelatin of the emulsion. In a mixed system two packets of different couplers may be incorporated in a single gelatin layer and a third coupler incorporated in another layer either directly in the emulsion or in dispersion in a solvent for the coupler. In a single emulsion layer, all three couplers may be in packets and the third coupler incorporated in a surrounding silver halide emulsion in the same layer. 60 Antistain agents other than diethylhydroquinone may be used in the emulsion such as diethylhydroquinone and didodecylhydroquinone.

65 It will be understood that the examples and modifications included herein are illustrative only and that the invention is to be taken as limited only by the scope of the appended claims.

We claim:

1. The method of making a packet photographic emulsion which comprises forming a mixture of (1) a non-diffusing color-forming compound capable of reacting with the oxidation product of a primary aromatic amino developing agent on photographic development and containing a group selected from the class consisting of sulfamylbenzamido, disulfamylbenzamido, alkylsulfamylbenzamido, dialkylsulfamylbenzamido, aminoalkylsulfamylbenzamido, diaminoalkylsulfamylbenzamido, hydroxylsulfamylbenzamido, dihydroxyalkylsulfamylbenzamido, phenylalkylsulfamylbenzamido, and diphenylalkylsulfamylbenzamido groups, (2) a gelatino-silver halide emulsion and (3) a water-soluble salt of a polymer se-

lected from the class consisting of methacrylic acid-methyl- $\alpha$ -methacrylate copolymer, algin, carboxymethyl cellulose and cellulose sulfate, said coupler being added to one of said other ingredients before the third ingredient is added, bringing the pH of the mixture below 7 immediately after adding said water-soluble salt, and adding to the mixture with stirring a solution of a polymeric carbon chain compound having recurring phenyl groups, carboxylic acid groups and amide groups to form a dispersion of particles of gelatin, packet-forming component and silver halide, containing said color-forming compound.

2. The method of making a packet photographic emulsion which comprises forming a mixture of (1) a non-diffusing coupler compound containing a hydroxyalkylsulfamylbenzamido group and capable of reacting with the oxidation product of a primary aromatic amino developing agent on photographic development, (2) a gelatino-silver halide emulsion and (3) a water-soluble salt of a copolymer of methacrylic acid and methyl- $\alpha$ -methacrylate, said coupler being added to one of said other ingredients before the third ingredient is added, bring the pH of the mixture below 7 immediately after adding said water-soluble salt, and adding to the mixture with stirring a solution of a water-soluble salt of an interpolymer of styrene and an  $\alpha,\beta$ -unsaturated carboxylic acid to form a dispersion of particles of gelatin, salt of said interpolymer and silver halide, containing said color-forming compound.

3. The method of making a packet photographic emulsion which comprises dispersing in gelatin a non-diffusing coupler compound containing a hydroxyalkylsulfamylbenzamido group and capable of reacting with the oxidation product of a primary aromatic amino developing agent on photographic development, mixing said coupler dispersion with a gelatino-silver halide emulsion, mixing with the emulsion and coupler mixture a solution of a water-soluble salt of a copolymer of methacrylic acid and methyl- $\alpha$ -methacrylate, bringing the pH of the resulting mixture below 7, and then adding to the mixture with stirring a solution of a water-soluble salt of an interpolymer of styrene and an  $\alpha,\beta$ -unsaturated carboxylic acid to form a dispersion of particles of gelatin, salt of said interpolymer and silver halide, containing said coupler compound.

4. The method of making a mixed packet photographic emulsion which comprises dispersing in gelatin a non-diffusing coupler compound containing a hydroxyalkylsulfamylbenzamido group and capable of reacting with the oxidation product of a primary aromatic amino developing agent on photographic development, mixing said coupler dispersion with a gelatino-silver halide emulsion sensitive to one region but less than all regions of the visible spectrum, mixing with the emulsion and coupler mixture a solution of a water-soluble salt of a copolymer of methacrylic acid and methyl- $\alpha$ -methacrylate, bringing the pH of the resulting mixture below 7, and then adding to the mixture with stirring a solution of the ammonium salt of styrene-maleic acid anhydride copolymer to form a dispersion of particles of gelatin, ammonium salt of

said copolymer and silver halide, containing said coupler compound, and forming in the same way as said last-mentioned dispersion at least one other dispersion of particles of gelatin, styrene-maleic acid anhydride copolymer, silver halide sensitive to a different region of the visible spectrum than said first-mentioned silver halide, and a non-diffusing coupler compound containing a hydroxyalkylsulfamylbenzamido group and capable of reacting with the oxidation product of a primary aromatic amino developing agent on photographic development different from said first-mentioned coupler compound, and mixing said dispersions of particles together.

5. The method of making a packet photographic emulsion which comprises mixing with a solution of a non-diffusing color-forming compound containing a hydroxyalkylsulfamylbenzamido group and capable of reacting with the oxidation product of a primary aromatic amino developing agent on photographic development a solution of a water-soluble salt of a copolymer of methacrylic acid and methyl- $\alpha$ -methacrylate, bringing the pH of the resulting solution below 7, mixing with the solution a gelatino-silver halide emulsion, and then adding to the resulting mixture with stirring a solution of a water-soluble salt of an interpolymer of styrene and an  $\alpha,\beta$ -unsaturated carboxylic acid to form a dispersion of particles of gelatin, salt of said interpolymer and silver halide, containing said color-forming compound.

6. The method of making a mixed packet photographic emulsion which comprises dispersing in gelatin a non-diffusing color-forming compound containing a hydroxyalkylsulfamylbenzamido group and capable of reacting with the oxidation product of a primary aromatic amino developing agent on photographic development a solution of a water-soluble salt of a copolymer of methacrylic acid and methyl- $\alpha$ -methacrylate, bringing the pH of the resulting solution below 7, mixing with the solution a gelatino-silver halide emulsion sensitive to one region but less than all regions of the visible spectrum, and then adding to the resulting mixture with stirring a solution of the ammonium salt of styrene-maleic acid anhydride copolymer to form a dispersion of particles of gelatin, salt of said copolymer and silver halide, containing said color-forming compound, and forming in the same way as said last-mentioned dispersion at least one other dispersion of particles of gelatin, styrene-maleic acid anhydride copolymer, silver halide sensitive to a different region of the visible spectrum than said first-mentioned silver halide, and a non-diffusing color-forming compound containing a hydroxyalkylsulfamylbenzamido group and capable of reacting with the oxidation product of a primary aromatic amino developing agent on photographic development different from said first-mentioned color-forming compound, and mixing said dispersions of particles together.

55      References Cited in the file of this patent

FOREIGN PATENTS

878,094      France ----- Sept. 28, 1942